

June 3, 1947.

H. B. KLINE ET AL

2,421,624

## METHOD OF CONDITIONING ARTIFICIAL SILK THREAD

Original Filed Oct. 9, 1941 3 Sheets-Sheet 1



June 3, 1947.

H. B. KLINE ET AL

2,421,624

## METHOD OF CONDITIONING ARTIFICIAL SILK THREAD

Original Filed Oct. 9, 1941 3 Sheets-Sheet 2



June 3, 1947.

H. B. KLINE ET AL

2,421,624

METHOD OF CONDITIONING ARTIFICIAL SILK THREAD

Original Filed Oct. 9, 1941 3 Sheets-Sheet 3



FIG. 3

HAYDEN B. KLINE  
KENNETH M. McLELLAN  
INVENTORS

BY *Frederick L. Birney*  
ATTORNEY

## UNITED STATES PATENT OFFICE

2,421,624

METHOD OF CONDITIONING ARTIFICIAL  
SILK THREAD

Hayden B. Kline and Kenneth M. McLellan,  
Cleveland, Ohio, assignors to Industrial Rayon  
Corporation, Cleveland, Ohio, a corporation of  
Ohio

Original application October 9, 1941, Serial No.  
414,325. Divided and this application July 13,  
1944, Serial No. 544,720

4 Claims. (Cl. 117—7)

1

This invention relates to the manufacture of filaments, bands, ribbons, thread and the like, hereinafter referred to as "thread"; particularly, artificial silk thread characterized by a high tensile strength.

This application is a division of application Serial No. 414,325, filed October 9, 1941.

Artificial silk thread, especially multiple filament viscose artificial silk thread, which is characterized by a high tensile strength is not easy to manufacture. When produced by ordinary methods, such thread is markedly nonuniform in its physical and physicochemical properties, varying noticeably not merely from batch to batch but even within the same batch. As a rule, excessive manipulation of the thread incident to the conventional process of manufacturing it results in undue waste of partially processed material.

In all usual methods of manufacturing multiple filament viscose artificial silk thread of high tensile strength, the necessary stretch is imparted to the thread only after it has had time to become set. A high stretch cannot be imparted to such thread without causing rupture of some of the filaments thereof, bringing about a concomitant reduction in the tensile strength of the thread as a whole. Prior art methods of stretching thread to increase its tensile strength have been seriously limited by this seemingly inherent inability of the thread to withstand more than a moderate amount of stretching.

The present invention not only simplifies the process as a whole but permits extremely high stretches to be imparted to the thread without detrimental effects upon its quality. This is accomplished by employing a plurality of stretching operations, such operations being performed on thread which has been treated so as to enhance its capacity for stretching. Preferably, the thread is in a somewhat plastic state when the stretching operations are performed upon it. Inasmuch as all operations, including stretching operations, are performed upon the thread in one continuous sequence, many of the difficulties found in prior art methods are obviated.

Apparatus suitable for the purposes of the invention comprises, among other things, a thread source, a catena of thread-advancing thread store devices upon each of which the thread is continuously but temporarily stored in substantially helical turns while the desired processing operations are performed upon it, and appropriate collecting means. After leaving the source, the thread passes in succession to each of the 50

2

several thread-advancing thread store devices comprising the catena. From the last thread-advancing thread store device of the catena, the processed thread passes directly to the collecting means.

Figure 1 of the drawings shows an end elevation of apparatus with which the invention may be employed, such apparatus embodying two oppositely inclined banks made up of laterally adjacent catenae. Figure 2 is a side elevation of the apparatus of Figure 1 from line 2—2 thereof showing in detail one of the inclined banks. Figure 3 is a substantial sectional elevation of the apparatus.

15 In the drawings, several laterally adjacent catenae individually made up of ten thread-advancing reels of cantilever construction are represented more or less diagrammatically. Actually, each reel in each catena comprises two cage-like reel members of substantially circular cross section which occupy substantially the same space, the periphery of each reel member being made up of a plurality of longitudinally extending thread-supporting bars. The bars of each 20 reel member interdigitate with and are alternately disposed with respect to the bars of the other reel member. The reel members of each reel rotate about axes displaced from each other, for instance, they may be and preferably are in 25 inclined relation in parallel planes.

30 The number of turns of thread per unit of length on a given reel is a function of the angle of inclination of the axes of rotation of the two reel members. Such angle of inclination is determined in part by the size of the thread to be 35 stored on the reel. As viewed from a plane parallel to the two parallel planes in which the axes lie, the apparent intersection of the axes of rotation of the two reel members may be at any point 40 along the reel as a whole but preferably near the center of the thread-bearing portion thereof. In the drawings, the number of turns of thread and the spacing between turns on the illustrated reels 45 are not to scale.

Reels of the type described and apparatus of the kind illustrated as embodying them are shown in Patent 2,225,642 to Walter F. Knebusch et al.

The laterally adjacent catenae going to make up the two oppositely inclined banks shown in Figure 1 are supported on each side of an A-shaped frame 12. In each catena, the unsupported end of each reel is directed toward the working face of the bank with which it is associated. Reels 2 to 10, inclusive, are disposed in

stepped relation as shown in Figures 1 and 3 with the thread-discharge portion of each reel in juxtaposition to the thread-receiving portion of the succeeding reel. Such an arrangement offers constructional and operative advantages which will appear more clearly hereinafter.

As shown in Figure 3, reels 1 and 2 may, if desired, be constructed with a flared contour so that thread being advanced therealong will be stretched as it is advanced. These reels need not necessarily be flared, for either or both may be substantially cylindrical. If desired, other reels included among reels 3 to 10, inclusive, may be of such flared contour; also, any of reels 3 to 10, inclusive, may be of tapered contour so that the thread may contract in passing therover. Preferably, however, reels 3 to 10, inclusive, are substantially cylindrical.

Reels 1 to 10, inclusive, are driven through change speed mechanism 14 by means of a motor 13 located at the "drive end" of the apparatus, i. e., the end at the left in Figure 2. Speed reduction unit 15, driven by change speed mechanism 14, actuates a drive shaft 16 extending longitudinally of the machine which shaft serves to drive all reels 1 through suitable gear boxes 17. In similar fashion, speed reduction unit 18, also driven by motor 13 through change speed mechanism 14, actuates the two longitudinally extending drive shafts 19 which, through gear boxes 21 and inclined drive shafts 22, serve to drive reels 2 to 10, inclusive.

Gears 23, mounted on inclined drive shafts 22, mesh with gears 24 mounted on reels 2 to 10, inclusive. Gears 23 and 24 are demountable, consequently, changes may be made in the speeds of reels 2 to 10, inclusive, by changing these gears. If desired, the gear ratios of the gears for each reel may be maintained constant and a peripheral speed differential between successive reels obtained by using successive reels of different diameters. In either case, successive reels in the catena may be rotated at peripheral speeds greater or less than preceding reels, thereby imparting stretch to or allowing for contraction of the thread, as the case may be, while it is passing from reel to reel.

By employing a driving arrangement of this kind, reels 1 and reels 2 to 10, inclusive, may be driven at different speeds by suitable adjustment of change speed mechanism 14. If it is desired to stop rotation of any reel 1, the corresponding clutch handle 25 may be turned to disengage the coupling through which such reel is driven from shaft 16. Similarly, any catena of reels 2 to 10, inclusive, may be stopped by operating clutch handle 26. If desired, one or more reels in each of the several catenae may be provided with a slip clutch device so that rotation of any one of the reels thus equipped may be interrupted without affecting the rotation of other reels in the catena.

Since the illustrated apparatus is adapted to produce the thread as well as to process it, a particularly convenient arrangement is one pursuant to which motor 13, through change speed mechanism 14, speed reduction unit 21 and shafts 28, drives gear pumps 29 disposed at intervals along the front of the apparatus. Gear pumps 29 are connected to spinning solution supply pipes 31 in such manner that a coagulable spinning solution, i. e., viscose, can be fed at a uniform rate through feed pipes 32 and pivotally mounted mass tubes 33 to spinnerets 34. As the spinning solution is extruded into precipitating

bath 35 in trough 36, it is coagulated to form a multiple filament artificial silk thread 37.

Liquid for coagulating the spinning solution as it is extruded into precipitating bath 35 is supplied to trough 36 from the end of the apparatus opposite the drive end. It passes to trough 36 through weir box 38, header boxes 39, and inlet pipes 41, which parts are connected together as shown in Figure 3. The coagulating liquid passes into trough 36 through orifices 42 disposed at intervals along inlet pipe 41. Inasmuch as there is preferably a continuous flow of coagulating liquid into coagulating trough 36, the excess liquid is permitted to pass therefrom through overflow pipe 43 and return pipe 44 to suitable make-up and recirculation means.

The freshly formed thread 37 passes substantially vertically upward from the precipitating bath to the thread-receiving end of reel 1, passing through thread guide 45. Guide 45 not only leads thread 37 to reel 1 but also serves to strip therefrom a considerable amount of the entrained coagulating liquid. Although a considerable quantity of coagulating liquid is stripped from thread 37 in this manner before it passes to reel 1, enough remains so that coagulation of the freshly formed thread continues while the thread is being advanced over the periphery of the reel.

It is sometimes desirable to apply an oleaginous material to reels 1 to inhibit deposition of deposits thereon; accordingly, oil supply pipes 46 and drip pipes 47 may be employed to drip oil or the like onto reels 1.

After thread 37 has been advanced to the thread-discharge end of reel 1, it passes from reel 1 vertically downward through channel 48, part of which is shown as broken away in order to show the path of the thread. From the lower end of channel 48 the thread passes under thread guide 51 or, as in Figure 3, under guide 51 and over thread guide 52. Guide 51 or 52, as the case may be, serves to locate the point at which thread 37 starts to wind onto the succeeding reel. For convenience, guide 52 is adjustably mounted to provide for the storage on reel 2 of varying amounts of thread.

Similar thread guides 53 are disposed between adjacent reels 2 to 10, inclusive; however, the thread usually passes between two adjacent reels in a substantially straight line.

The thread is subjected to the desired processing operations as it advances in closely spaced, substantially helical turns over each of reels 2 to 10, inclusive. Collecting troughs 56 are disposed beneath each horizontal series of reels 2 to 10, inclusive, to collect any excess of the liquid applied to the thread: these troughs operate to return the collected liquid through outlets 57. Troughs 56 have formed therein near the forward edges thereof supply conduits 58 adapted to conduct processing liquid through distributor pipes 55 to the reels in the horizontal series disposed immediately below each of such troughs. A pipe 54 extends longitudinally of the apparatus above reels 2 to supply suitable treating liquid through distributor pipes 55 to the thread 37 stored on reels 2.

Ordinarily, only one set of conditions is employed at one time on one and the same apparatus; for this reason, the left and right-hand banks appearing in Figure 3 constitute images of each other.

After having been processed as desired on reels 1 to 7, inclusive, the thread on reaching reel 8 is

treated with an oil emulsion to enhance its flexibility in preparation for the twisting operation. In order that no unnecessary excess emulsion will remain on the thread, reel 9 is utilized as a drip stage. As will hereinafter appear, the ratio of the peripheral speed of reel 8 to that of reel 9 affects the effectiveness of the drip stage. The latter is intended to accomplish the removal of a substantial amount of the liquid which would otherwise cling to the thread; indeed, by the time the thread reaches the discharge end of reel 9, it should have a comparatively low, constant moisture content so that it may be dried without undue difficulty.

Reels 10, on which the thread is dried, may be heated internally by hot water, oil, steam, etc. to a temperature high enough to dry the threads substantially completely but in any event to an extent sufficient to permit it to be collected in finished form on cap twisters 62, to which the threads proceed through thread guides 61 after leaving the unsupported end of reels 10. Ordinarily, a temperature of 80° C. to 100° C. is sufficient to accomplish the drying of the thread in a reasonable time. Reels suitable for drying multiple filament artificial silk thread of the kind to which the present invention relates are shown, described and claimed in Jordan Patent 2,207,739.

Cap twisters 62 are disposed below the horizontal series of reels 10, one cap twister being associated with each descending catena of reels 1 to 10, inclusive.

Motor 63 actuates the cap twisting mechanism through cam 64 and cam-following lever 65 which effects vertical reciprocation of lifter rail 66. The same motor 63 actuates driving drum 67 around which whorl belt 68 passes. While lifter rail 66 reciprocates in a vertical direction, whorls 69 are rotated by belt 68 which passes therearound. Thus the thread passing to the cap twister 62 is simultaneously twisted and collected on bobbins 70. Shields 71 are disposed between adjacent cap twisters 62 to prevent entanglement of the respective threads 37 as they "balloon" about the cap twisters, such shields being attached to the bottom of housings 72 which enclose dryer reels 10.

Although the invention may be employed in the manufacture of other types of artificial silk thread, it will be described hereinafter as applied to the manufacture of viscose artificial silk thread having a dry tensile strength of at least 2.5 grams per denier.

A thread of relatively high tensile strength may be produced by subjecting it in the early stages of regeneration to a plurality of successive stretching operations each of which stretches the thread but none of which is great enough to break the filaments of which the thread is composed. In this state, i. e., before regeneration proceeds to completion, an inherent tendency to contract exists in multiple filament viscose artificial silk thread, regardless of whether it is passing along the peripheries of the reels or passing between reels.

If, for example, the peripheral speeds of reels 1 and 2 are the same, a normal tension due entirely to the aforementioned inherent tendency to contract will exist in the thread, which tension may be as much as 50 grams or more as measured by a thread deflection tensiometer. A similar tension exists in the thread passing between reels 2 and 3 even if the peripheral speeds of those reels are equal. A like state of affairs obtains in varying degrees on and between the subsequent reels of each catena. This normal tension is to

be distinguished from tensions introduced by stretching operations as hereinafter described.

In these circumstances, if two or more stretching operations are introduced, the tension developed in viscose artificial silk thread during the later of two stretching operations will be much greater than that developed during the earlier stretching operation, without regard to the fact that the second may not be as drastic as the first. 5 Not only this, but where two or more stretching operations are employed, the total tension in the thread in a given stretching stage, i. e., that tension induced by the stretching operation together with the tension due to the inherent tendency of the thread to contract, will vary in different stretching stages even though the magnitude of the respective stretching efforts may be the same.

The inherent contraction of viscose artificial silk thread is dependent upon a number of factors including the amount of stretching in the preceding stages and the length of elapsed time between extrusion and stretching. The amount of inherent contraction may, however, be increased, decreased, or otherwise controlled by subjecting the thread to certain processing treatments before or during the stretching operations. Among other things, it is possible to provide thread of comparatively high tensile strength by reducing inherent contraction to a minimum in at least one of a plurality of stretching operations while imparting the desired amount of stretch to the thread.

When, for instance, the thread is stretched between reels 1 and 2, the inherent tendency to contract limits the extent to which the thread may be stretched. Likewise, inherent contraction limits the amount of stretch which can normally be imparted between reels 2 and 3. Accordingly, before the thread is stretched between reels 2 and 3, it is preferably conditioned as hereinafter described so as to render it capable of being stretched to the desired extent without deleteriously affecting the individual filaments of which the thread is composed.

45 For the most part, best results are obtained when the highest tension developed in any of a plurality of separate stretching stages is maintained at a minimum, this being achieved by applying to the thread, preferably immediately 50 prior to the stage in which such tension is developed, a suitable treating fluid at a temperature between 10° and 60° C. The medium applied to the thread may be water or other treating fluid, for example, an aqueous solution of a strong 55 acid. If water is employed, it is desirable to treat the thread for a somewhat longer period of time or at a somewhat higher temperature than if an acid is used. The length of time of treatment may be increased or decreased by increasing 60 or decreasing the number of turns of thread on the reel.

The methods described herein may also be performed in the absence of the step of continuously but temporarily storing the freshly formed thread on reel 1.

In the following example, the freshly formed thread travels a distance of approximately fifteen inches in the coagulating bath and approximately 70 26 inches in the air before it comes into contact with the first reel of the catena. The distance between the point at which the thread leaves the first reel and that at which it winds onto the second reel is approximately eighty-one inches. The distance between succeeding reels 75 is approximately nine inches. The length of

thread stored on each reel varies as indicated in the example.

*Example*

As shown in Figure 3, thread 37 is drawn vertically upward out of the coagulating bath by a flared reel 1 which imparts a stretch of approximately 15% to the freshly formed thread as it advances thereover from the supported to the unsupported end of the reel.

At the thread-receiving end of reel 1, the peripheral speed thereof is 43.7 meters per minute, while at the thread-discharge portion thereof, the peripheral speed is 50.3 meters per minute. Additional stretch is imparted to the thread as it passes between reels 1 and 2, the latter having, for instance, a peripheral speed of 58.8 meters per minute at the thread-receiving end thereof. A third stretch is imparted to the thread as it advances over the periphery of flared reel 2, which has a peripheral speed at its thread-discharge end of 67.7 meters per minute. Reels 3 to 8, inclusive, rotate at a peripheral speed the same as that of reel 2 at the thread-discharge end thereof; viz., 67.7 meters per minute.

When a liquid is applied to the thread stored on reel 2 as hereinafter explained, the thread passing between reels 1 and 2 preferably has approximately 110 grams tension, while that passing between reels 2 and 3 preferably has 80 grams tension.

Under preferred conditions, no processing liquid is applied to the thread stored on reel 1 but a dilute acid solution comprising water, 2.5%  $H_2SO_4$ , 5%  $Na_2SO_4$  and 0.05%  $ZnSO_4$  is applied at a temperature of 30° C. and at a rate of approximately 300 c. c. per minute to the thread stored on reel 2. The application of the treating liquid to the thread stored on reel 2 not only increases the ability of the thread to withstand greater stretching but also reduces the inherent tension in the thread during and after the stretching operation. The same treating solution is applied to the thread while it is being advanced on reel 3, the temperature and rate of application being the same as that applied to the thread on reel 2. From the thread-discharge end of reel 3 the thread passes to the thread-receiving end of reel 4, where approximately 60 turns of thread are stored while a faintly acid aqueous washing liquid (.02%  $H_2SO_4$ ) is applied to the thread at a temperature of 30° C.

The thread is then passed from reel 4 to reel 5 where it is stored in approximately 70 turns while fresh water is applied thereto at a temperature of 30° C. to wash free of excess acid, salts, etc.

If it is found desirable to remove the sulphur contained in the thread by a desulphurizing process, the thread is passed to reel 6, upon which approximately 60 turns of thread may be stored while a .35% aqueous solution of sodium sulfide is applied thereto at a temperature of 50° C. While it is not in all cases necessary to employ such a desulphurizing operation, if it is employed, the excess of such desulphurizing solution should be washed from the thread on reel 7. The thread is stored upon reel 7 in approximately 60 turns while water is applied thereto at a temperature of 30° C.

The twisting operation to which the thread is subjected in the final stage requires a certain amount of lubrication of the thread. Accordingly, thread 37 passes from reel 7 to reel 8, where an oil emulsion is applied to the thread while approximately 60 turns of thread are stored thereon.

The emulsion may consist of a mixture of mineral oil and a sulfonated hydrocarbon dispersed in an aqueous medium. The emulsion applied to the reel is preferably maintained at a temperature of approximately 40° C.

Since it is undesirable to have an undue amount of moisture in the thread immediately prior to the drying operation, reel 9 acts as a "drip" stage for the thread: in such stage, approximately 36 turns of thread are stored on the reel.

It has been found that by decreasing the peripheral speed of reel 9 with respect to that of reel 8; for instance, by making the diameter of reel 9 less than that of reel 8 while maintaining the angular velocity the same as that of reel 8, more liquid can be removed from the thread in the drip stage than if the peripheral speeds of the two reels were equal or if the peripheral speed of reel 9 were greater than that of reel 8. For this surprising state of affairs no satisfactory explanation is available at the present time. Ordinarily a reduction of approximately 2% in peripheral speed is sufficient to achieve the desired results.

The optimum percentage of reduction in peripheral speed usually is determined by the amount of tension which has been developed in the thread during the previous stages. For example, if the peripheral speed of reel 8 is 67.7 meters per minute and a total stretch of 55% has been imparted to the thread in the first stages of regeneration, reel 9 should have a peripheral speed of approximately 66.4 meters per minute. In general, the greater the amount of tension developed in the thread during the stretching operation, the greater should be the difference in peripheral speeds of reels 8 and 9.

In order that the desired residual shrinkage and elongation properties may be imparted to the finished thread, the moist thread is stretched slightly while it passes from the thread discharge end of drip reel 9 to the thread-receiving end of drying reel 10. Preferably the amount of stretch imparted to the thread between reels 9 and 10 is less than the amount of let-off in the thread between reels 8 and 9. In the instant example, drying reel 10 should have a peripheral speed of approximately 67 meters per minute, whereby approximately 1% stretch is imparted to the thread while it passes from reel 9 to reel 10. Of course, the peripheral speeds of the reels may be varied in any desirable manner such as decreasing the speed of the intermediate reel and increasing the speed of the drying reel over both previous reels or either one, depending on the final required yarn characteristics.

Drying reel 10 may be heated to a temperature of 85-90° C. by hot water, oil or other suitable heating fluid while approximately 100 turns of thread are stored thereon. Inasmuch as reel 10 is substantially cylindrical and the thread is restrained somewhat from shrinking during the drying thereof, the dried thread may have a residual capacity to shrink of 6% or more based on the original length of the finished thread. Since the shrinkage is uniform throughout all parts of the thread, the quality thereof is not in any way lowered because of such relatively high residual shrinkage capacity.

The dried thread is collected on cap-twisting apparatus of the type hereinbefore described, approximately two and one half turns per inch twist being imparted to the thread.

Thread manufactured according to the pre-

cedure hereinbefore set forth has the following physical properties:

| Denier | Filaments | Elongation       | Shrinkage        | Wet Tensile   | Dry Tensile   |
|--------|-----------|------------------|------------------|---------------|---------------|
| 275    | 120       | Per cent<br>10.6 | Per cent<br>6.79 | G./d.<br>1.85 | G./d.<br>3.31 |

Under similar conditions, a thread of 100 denier, 40 filaments, may be produced by decreasing the delivery rate of the viscose pumps to 7.8 grams per minute. The physical properties of such thread are:

| Denier | Filaments | Elongation      | Shrinkage        | Wet Tensile   | Dry Tensile   |
|--------|-----------|-----------------|------------------|---------------|---------------|
| 100    | 40        | Per cent<br>9.3 | Per cent<br>6.75 | G./d.<br>1.89 | G./d.<br>3.20 |

Since thread of the latter type will require less spacing between turns on the respective reels, the following table may be taken as giving the preferred number of turns of thread to be stored on the reels.

|         |     |
|---------|-----|
| Reel 3  | 90  |
| Reel 4  | 120 |
| Reel 5  | 140 |
| Reel 6  | 140 |
| Reel 7  | 140 |
| Reel 8  | 120 |
| Reel 9  | 36  |
| Reel 10 | 100 |

Also, the inherent contraction and total tensions will be only about  $\frac{1}{3}$  of the values stated for a thread of 275 denier, 120 filaments.

Although thread-advancing reels are preferred for the purposes of the invention, it is possible to substitute therefor sets of inclined, spaced rollers, particularly in handling freshly spun thread. At points where only one or two turns of thread are to be handled, it is possible to employ godet wheels. If, however, a processing medium is to be applied to the thread or if it is desired to store the thread for a relatively long time, thread-advancing reels of the type illustrated are preferred, principally because a large number of turns may be stored thereon in a small space. Numerous other modifications may be made in the methods and apparatus herein described without departing from the spirit of the invention.

It is intended that the patent shall cover, by suitable expression in the appended claims, whatever features of patentable novelty reside in the invention.

We claim:

1. The method of processing regenerated cellulose artificial silk thread comprising applying a liquid to the thread while it is continuously but temporarily stored on a first thread store device in a plurality of substantially helical turns, passing the wet thread to a second thread store de-

vice upon which the thread is stored continuously but temporarily in a plurality of substantially helical turns and to which thread no further liquid is applied, and rotating said second thread store device at a peripheral speed less than that of said first thread store device whereby the liquid carried by the thread from said first device drips from the thread, said steps being performed in a continuous sequence of operations.

2. The method of processing regenerated cellulose artificial silk thread comprising applying a liquid to the thread, continuously but temporarily storing the wet thread on a first thread store device in a plurality of substantially helical turns, passing the wet thread to a second thread store device upon which the thread is continuously but temporarily stored in a plurality of generally helical turns, rotating the second thread store device at a peripheral speed less than the peripheral speed of said first thread store device, passing the moist thread to a thread store device adapted to store the thread continuously but temporarily during drying thereof; and rotating the drying device at a peripheral speed greater than that of said second thread store device, said steps being performed in a continuous sequence of operations.

3. The method described in claim 2 wherein the peripheral speed of the drying device is greater than that of said first device.

4. The method of manufacturing viscose artificial silk thread comprising applying a liquid-processing medium to the thread while said thread is being continuously but temporarily stored upon a thread store device in substantially helical turns, drawing the wet thread from said thread store device by means of a succeeding thread store device which has a peripheral speed less than the former device, advancing the thread over the periphery of said succeeding thread store device in a plurality of substantially helical turns while no liquid-processing medium is applied to the thread stored thereon, drawing the moist thread from said succeeding thread store device to a thread store device adapted to dry the moist thread, said thread store device adapted to dry the thread having a peripheral speed greater than that of said succeeding thread store device but less than the first-mentioned thread store device, said steps being performed in a continuous sequence of operations.

HAYDEN B. KLINE.  
KENNETH M. MCLELLAN.

#### REFERENCES CITED

The following references are of record in the file of this patent:

#### UNITED STATES PATENTS

| Number    | Name               | Date         |
|-----------|--------------------|--------------|
| 2,189,195 | Burkholder         | Feb. 6, 1940 |
| 2,002,996 | Hoefinghoff et al. | May 28, 1935 |